

No. 874,641.

PATENTED DEC. 24, 1907.

W. TAYLOR.  
APPARATUS FOR USE IN THE HARDENING OF STEEL.  
APPLICATION FILED MAR. 11, 1907.



Fig. 1.



Fig. 2.

Witnesses:

J. B. Keay

C. D. Messler

Inventor

William Taylor

James L. Morris

Attest

# UNITED STATES PATENT OFFICE.

WILLIAM TAYLOR, OF LEICESTER, ENGLAND.

## APPARATUS FOR USE IN THE HARDENING OF STEEL.

No. 874,641.

Specification of Letters Patent.

Patented Dec. 24, 1907.

Application filed March 11, 1907. Serial No. 361,794.

*To all whom it may concern:*

Be it known that I, WILLIAM TAYLOR, a subject of the King of Great Britain, residing at Stoughton Street Works, Leicester, in the county of Leicester, England, engineer, have invented certain new and useful Improvements in Apparatus for Use in the Hardening of Steel, of which the following is a specification.

It is known that in hardening, tempering, or annealing steel, the proper quenching temperature for many purposes is one at which recalescence occurs, and it is important that this temperature, which varies between fairly wide limits with different samples of steel, should not be seriously exceeded. It is also known that at the recalescence temperature the permeability of iron or steel falls more or less suddenly to unit value, the material becoming non-magnetic, and this is true more particularly when the magnetic induction or flux density in the material is small.

The present invention relates to apparatus in which this change in the magnetic properties of the material at the critical temperature is utilized to call the attention of the workman to the fact that this temperature has been reached by a mass of steel which is being heated for the purpose of annealing, tempering, or hardening it by quenching, or it may be to release the said mass of steel so that it drops automatically into the quenching bath when this temperature is reached.

The apparatus hereinafter described is more particularly applicable to the hardening of small masses of steel in the form of bars or rods, such as for example small drills or taps, for which purpose the mass of steel to be treated is held suspended by magnetic attraction across or between soft iron polar extensions of a magnet, and is heated by a flame or other suitable source of heat. When the mass reaches the proper temperature for quenching it is automatically dropped from both poles into the quenching bath, or if it be desired to heat and harden one end only of the rod it will be released from the polar extension which is nearer to the heated end and hang suspended from the other polar extension, thereby indicating that the quenching temperature has been reached.

In order to prevent the piece of steel when released from one polar extension, herein after called the releasing pole, being jerked off the other extension, the surface of the

latter, hereinafter called the retaining pole, is curved.

The polar extensions consist of rods of soft iron or mild steel preferably of circular section and comparatively small diameter so that the surface of contact between the mass of steel and the pole pieces is small in order to avoid the liability to local chilling and for this purpose when slender pieces of steel have to be treated one or both of the polar extensions may be still further reduced towards the point of contact with the steel, as by tapering it towards its free end.

In the accompanying drawings, Figure 1 is an elevation partly in section of the most convenient form of apparatus adapted for heating the work in an open flame, and Fig. 2 illustrates a modified arrangement adapted for heating the steel in a lead or other bath.

In these drawings *a* is a permanent magnet, having soft iron polar extensions *b* *b*<sup>2</sup> one or both of which may be cranked or bent and rotatably secured at one end in the poles *a* *a*<sup>2</sup> respectively of the magnet, which for this purpose may be provided with clamp screws as shown in the drawing or with other equivalent device. This construction enables the distance between the outer ends of the polar extensions to be adjusted to take masses of steel of different lengths. The magnet may be either an electromagnet or a permanent magnet as shown.

With the apparatus shown in Fig. 1, the mass of steel *c* to be hardened is supported magnetically across the soft iron extensions *b* *b*<sup>2</sup> in contact with their lower sides as shown in the drawing, and is heated by the application of a flame or other suitable source.

If it is desired to harden only one end of the mass of steel, that end is placed in contact with the releasing pole *b*<sup>2</sup> which for this purpose is of varying section and permits of choosing a point of contact which is on the one hand sufficiently large to support the mass, but which on the other hand is not so large as to be liable to chill the mass locally. This end of the mass having reached the critical temperature, will be released by the pole *b*<sup>2</sup> and the mass will hang suspended in an approximately vertical position from the retaining pole *b* the surface of which is curved so that the mass of steel shall not be jerked therefrom by encountering any sudden irregularity of its surface.

When the mass of steel is heated out of

contact with the air as shown in Fig. 2, in a bath *d* of molten lead or other fluid of greater density than the steel, it will rise to the surface of the bath automatically, with or without the assistance of a spring *e* or equivalent counterweight, when it becomes non-magnetic, and it is to be understood that the term "magnetic support" hereinafter used in the claims is to be construed as applying to 10 such an arrangement as well as to the case in which the mass of steel falls down by gravity when released by its magnetic support.

Having thus described the nature of my 15 said invention and the best means I know of carrying the same into practical effect, I claim:—

1. An apparatus applicable to the hardening, tempering or annealing of steel, comprising a magnet having polar extensions of soft 20 iron rigidly connected therewith, said extensions being adapted to support magnetically the mass of steel under treatment and means for varying the distance between said polar extensions.
2. An apparatus applicable to the hardening, tempering or annealing of steel, comprising a magnet having polar extensions of soft iron adapted to be rotated so as to vary the 25 distance between said polar extensions and to be rigidly fixed in the poles of said magnet, said extensions being adapted to support magnetically the mass of steel under treatment.
3. In hardening, tempering or annealing 30 steel, an apparatus comprising a magnet having soft iron pole pieces extending normally parallel with each other, clamping screws in the poles of said magnet adapted to secure said pole pieces against rotation and said 35 pole pieces adapted by rotation in the poles of said magnet to vary the distance between the said pole pieces.
4. In hardening, tempering, or annealing 40 steel, an apparatus comprising a horse-shoe magnet, soft iron pole pieces extending normally in line with the limbs of said magnet 45 clamping screws in the poles of said magnet

adapted to secure said pole pieces against rotation and said pole pieces adapted by rotation in said limbs to vary the distance between the said pole pieces. 50

5. In hardening, tempering or annealing steel, an apparatus comprising a magnet having soft iron polar extensions, one of which is cranked and rotatably connected 55 with the magnet.

6. In hardening, tempering, or annealing steel, an apparatus comprising a magnet having soft iron polar extensions, said polar extensions being cranked and rotatably connected 60 with the magnet.

7. In hardening, tempering or annealing steel, an apparatus comprising a magnet having polar extensions, one of which has its surface curved to form a retaining pole. 65

8. In hardening, tempering or annealing steel, an apparatus comprising a magnet having soft iron polar extensions, one of which has its cross section gradually reduced toward its outer end to form a releasing pole. 70

9. In hardening, tempering or annealing steel, an apparatus comprising a magnet having soft iron polar extensions of circular section, one of which is of reduced diameter toward its outer end. 75

10. In hardening, tempering, or annealing steel, an apparatus comprising a magnet having a releasing pole of varying cross section, and a retaining pole of curved cross section, and means for varying the separation of the 80 poles.

11. In hardening, tempering or annealing steel, an apparatus comprising a bath for fluid, and a magnet adapted to hold therein magnetically the mass of steel under treatment. 85

In testimony whereof I have signed my name to this specification in the presence of two subscribing witnesses.

WILLIAM TAYLOR.

Witnesses:

A. PIERCE,  
H. P. HAGON.